

# UNITED STATES PATENT OFFICE.

OTTO DIETSCHÉ, OF BERLIN-LICHTENBERG, GERMANY, ASSIGNOR, BY MESME ASSIGNMENTS, TO THE CHEMICAL FOUNDATION, INC., A CORPORATION OF DELAWARE.

## PROCESS OF SEPARATING THORIUM FROM THE OTHER METALS OF THE RARE EARTHS.

1,835,157.

Specification of Letters Patent. Patented Mar. 30, 1920.

No Drawing.

Application filed April 15, 1915. Serial No. 21,533.

*To all whom it may concern:*

Be it known that I, OTTO DIETSCHÉ, a German citizen, and resident of Berlin-Lichtenberg, Germany, have invented certain new and useful Improvements in Processes of Separating Thorium from the other Metals of the Rare Earths, of which the following is a specification.

This invention relates to a novel process of separating thorium from the other metals of the rare earths by precipitating the same by means of hydrofluoric acid or by means of soluble fluorids.

If a solution of the metals of the rare earths is precipitated by means of soluble fluorids or by means of hydrofluoric acid, in general all metals of the rare earths will precipitate as fluorids; if however the precipitation is carried out only with a small quantity of the precipitating agent, thorium will precipitate first, while the other metals of the rare earths will precipitate only in a small quantity. The precipitation therefore is preferably carried out with a quantity of the precipitating agent which corresponds approximately to the content of thorium.

For solutions of a composition which is not accurately known it is preferable to carry on the process in such a manner that only small quantities of the precipitating agent (presumably less than an equivalent of the thorium) are added in succession and that the deposits are examined regarding their content of thorium.

If the deposit possesses too large contents of other metals of the rare earths the further precipitation is interrupted.

If one has frequently to do with solutions of essentially the same composition then it is preferable to find the most favorable conditions of precipitation and to carry on the process according to these conditions.

In order to obtain still purer thorium from the deposit which contains thorium in rather great quantities, the deposit may be redissolved anew and precipitated in the same manner. This process can be repeated as often as it appears desirable in the individual case. Also the deposit which contains great quantities of thorium may be further treated in another way.

The solutions of the metals of the rare earths from which the process originates may be of a different kind. Most preferably the chlorids or the nitrates are em-

ployed because with these there exists the least tendency for formation of double salts. It is however also possible to use for instance the sulfates. The transformation takes place in acid as well as in neutral solutions and both in cold and warm condition. The most favorable working conditions can be ascertained for each individual case according to the given solution.

In the following I desire to give an example of carrying my invention into effect:

100 kg. of a solution of the chlorids whose content of thorium corresponds to 2.5 kg. of thoric oxid, while the contents of the other earths amount to 25 kg., are mixed with 1.7 kg. of fluorid of sodium which is preferably dissolved in the necessary quantity of water and which is slowly added while keeping the mass in motion. The deposit contains about 70% thoric fluorid and 30% fluorids of the other earths while the ratio of thoric oxid and the other earths in the original solution had been about 1 : 10.

If it is not desirable to quantitatively separate the thorium, by reducing the quantity of sodium fluorid, the process may be carried on in such a manner that as early as the first precipitation approximately pure thorium fluorid will be obtained.

In case of using hydrofluoric acid as precipitating agent the process is carried out in an entirely analogous manner.

Having thus described my invention I claim as new and desire to secure by Letters Patent of the United States:—

1. A process for separating thorium from the other metals of the rare earths, which consists in reacting upon a solution of the metals of the rare earths with a quantity of a soluble fluorin compound substantially corresponding to the quantity of thorium contained in the solution.

2. A process for separating thorium from the other metals of the rare earths, which consists in precipitating a solution of the metals of the rare earths by means of fluorid of sodium, the quantity of said fluorid being chosen to result mainly in the precipitation of thorium contained in said solution.

3. A process for separating thorium from the other metals of the rare earths, which consists in precipitating a solution of the metals of the rare earths by means of a soluble fluorin compound of proper quantity to result mainly in a precipitation of the

thorium in said solution, thereupon dissolving the precipitated product, and again precipitating the same for further removing the other metals of the rare earths.

- 5 4. A process for separating thorium from the other metals of the rare earths, which consists in precipitating a solution of the metals of the rare earths by means of a soluble fluorid, the quantity of said fluorid being chosen to result mainly in a precipitation of the thorium in said solution, thereupon dissolving the precipitated product, and again precipitating the same for further removing the other metals of the rare earths.
- 10 10 5. A process for separating thorium from the other metals of the rare earths, which

consists in precipitating a solution of the metals of the rare earths by means of fluorid of sodium, the quantity of said fluorid being chosen to result mainly in a precipitation of 20 the thorium in said solution, thereupon dissolving the precipitated product, and again precipitating the same for further removing the other metals of the rare earths.

In testimony whereof I have hereunto set 25 my signature in the presence of two subscribing witnesses.

OTTO DIETSCHE.

Witnesses:

WALDEMAR HAUPT,  
HENRY HASPER.